

# UNITED STATES PATENT OFFICE.

CHARLES J. BARRENPOHL, OF NEW YORK, N. Y.

## COMPOUND FOR CLEANING AND POLISHING WOOD SURFACES.

No. 847,226.

Specification of Letters Patent.

Patented March 12, 1907.

Application filed December 19, 1906. Serial No. 348,504.

*To all whom it may concern:*

Be it known that I, CHARLES J. BARRENPOHL, a citizen of the United States, and a resident of the city of New York, borough of 5 Manhattan, county and State of New York, have invented a new and Improved Compound for Cleaning and Polishing Wood Surfaces, of which the following is a full, clear, and exact description.

This invention is an improved composition of matter for cleaning and polishing wood surfaces of all kinds having for objects, primarily, to produce a compound that will not only effectually remove finger-marks and 15 other collected dirt without affecting the wood, but will simultaneously with its application give the surface a high retaining polish and in addition close up the small openings in the grain of the wood, thus performing the function of a "wood-filler."

I accomplish the above objects by my cleaning and polishing compound, consisting of whiting, crude oil, lard-oil, and paraffin-wax combined in the following proportions 25 and in the manner hereinafter outlined: In any suitable vessel is placed one pound of paraffin-wax, which is heated until the same is entirely liquefied. To this is thereafter added three and one-half pints of crude oil— 30 as, for example, petroleum—and three and one-half pints of lard-oil, which are well mixed, when twenty-one and one-third pounds of whiting are added, and the whole stirred until the ingredients are thoroughly 35 intermingled, when the compound is ready for use.

The compound is applied to the surface of the wood by rubbing it on with a cloth or other device, the whiting acting to cut the

dirt, which is softened and dissolved by the 40 crude oil. The lard-oil gives the crude oil a body and renders the polish given by the compound harder and more lasting. The wax gives the surface a high polish, for which purpose it is added. The whiting in addition to cutting the dirt from the surface of the wood enters the small cracks, crevices, &c., in the grain of the same and provides an effectual wood-filler. In this connection the 45 whiting may, if desired, be colored by any 50 suitable pigment in order that it may harmonize with the wood on which it is used.

Although the proportions of ingredients hereinbefore indicated are found to give the best results, I regard the colorable variations as falling within the scope of my invention. 55

Having thus described my invention, I claim as new and desire to secure by Letters Patent—

1. The herein-described compound for 60 cleaning, filling and polishing wood surfaces, containing whiting, lard-oil and crude oil, combined in substantially the proportions set forth.

2. The herein-described compound for 65 cleaning, filling and polishing wood surfaces, consisting of whiting, lard-oil, crude oil and paraffin-wax, combined in substantially the proportions set forth.

In testimony whereof I have signed my name to this specification in the presence of two subscribing witnesses.

CHARLES J. BARRENPOHL.

Witnesses:

W. W. HOLT,  
JNO. M. RITTER.